

Dec. 28, 1937.

D. R. MERRILL ET AL.

2,103,591

PROCESS FOR PRODUCTION OF LUBRICATING OIL

Filed Oct. 24, 1932



## UNITED STATES PATENT OFFICE

2,103,591

## PROCESS FOR PRODUCTION OF LUBRICATING OIL

David R. Merrill, Long Beach, and Philip Subkow, Los Angeles, Calif., assignors to Union Oil Company of California, Los Angeles, Calif., a corporation of California

Application October 24, 1932, Serial No. 639,341

12 Claims.

(Cl. 196—13)

This invention relates to a process for the production of lubricating oil. More specifically it relates to a process for the production of lubricating oil from petroleum by the use of solvents.

One of the distinctive characteristics of a lubricating oil is its viscosity. Its usefulness as a lubricant depends, at least in part upon its viscosity. For many purposes lubricants are desired whose viscosity will vary as little as possible with variations in temperature, i. e. have low temperature viscosity susceptibilities. Those fractions which exhibit a low temperature viscosity susceptibility are oftentimes referred to as the paraffinic oils whereas the fractions which exhibit a high temperature viscosity susceptibility are referred to as the non-paraffinic oils.

The heavy oil fractions of many crude oils, from which lubricating oils are produced consist of a mixture of hydrocarbons some of which exhibit a low temperature viscosity susceptibility, some of which exhibit an intermediate temperature viscosity susceptibility, and some of which exhibit a high temperature viscosity susceptibility. In order to produce superior lubricating oil from hydrocarbon mixtures, as described above, those oils present having a high viscosity temperature susceptibility, and those having an intermediate temperature viscosity susceptibility are separated from the oils present which exhibit a low temperature viscosity susceptibility. Solvent extraction is one of the methods employed to separate the undesirable oil from the desirable oil. Solvents, such as aniline, furfural, nitrobenzene, selenium oxychloride, sulphur dioxide or B B' dichlorethyl ether are capable, under the proper conditions of temperature and pressure, of dissolving the fractions present which are non-paraffinic in character. The foregoing solvents under proper conditions of temperature and pressure are capable of dissolving the oils present in the hydrocarbon mixture which exhibit intermediate and high temperature viscosity susceptibilities. These oils dissolved in the solvent may be separated from each other by cooling in which case the oils exhibiting the intermediate temperature viscosity susceptibility are forced out of solution.

These solvents form relatively heavy solutions with the non-paraffinic oil fractions and can be separated from the insoluble paraffinic oil fractions by settling. The separated paraffinic oil fractions or raffinates and non-paraffinic oil fractions or extracts dissolved in solvent are then distilled to separate the solvent from the oil.

55 The paraffinic fractions may then be given such

further treatment as necessary to remove any remaining impurities. The non-paraffinic oil fractions being relatively valueless are utilized as fuel or as cracking stock in conversion processes.

The separation of hydrocarbon mixtures into paraffinic and non-paraffinic fractions by the use of solvents is not restricted to batch operation but may be carried out in a continuous manner. Where continuous extraction is employed it is customary to flow the solvent countercurrently to the oil to be extracted. Hence the oil being purified is progressively being contacted with solvent which is less contaminated with non-paraffinic fractions. The oil entering the extraction system is contacted with solvent containing a relatively high concentration of non-paraffinic fractions whereas the purified oil is finally contacted with pure solvent. In this manner the maximum degree of refinement is usually obtained because at the final stage of the extraction relatively pure oil is contacted with fresh solvent which has a high selective solvent power to separate the paraffinic and non-paraffinic fractions because it is not contaminated with non-paraffinic oil. When continuous countercurrent extraction is employed the extraction step may be carried out in one stage wherein the solvent and oil flow countercurrently or it may be carried out in a plurality of stages wherein the extracts obtained from the later stages of the process are returned to the earlier stages of the process and employed therein as the extracting medium. Thus in the first extraction stage the oil to be extracted is contacted with solvent containing dissolved fractions from a later stage. The insoluble oil portion in the first stage passes to the second stage where it is contacted with solvent containing less of the extracted fractions. The insoluble oil from the second stage passes successively in the same manner as described above, to the remaining extraction stages until it reaches the final stage wherein it is extracted with pure solvent. In processes of this character the same temperature is employed throughout the system and as final products there are obtained a fraction consisting largely of the non-paraffinic fractions and a fraction which is in the main composed of the paraffinic fractions.

We have found it more desirable to carry out the extraction of hydrocarbon mixtures containing paraffinic and non-paraffinic fractions countercurrently in a plurality of stages maintained at different temperatures and to separate from each stage a raffinate fraction. In such case the oil to be treated is contacted in the first

stage at a relatively high temperature with solvent containing extracted fractions obtained from the second extraction stage in which the extraction has been carried out at a lower temperature than the extraction in the first stage. A raffinate and extract are separated in the first stage. The extract is passed through a cooler to lower the temperature upon which a further separation of oil and extract takes place. The cooled mass is then passed to a column where the extract settles out and is withdrawn. The insoluble oil in this column passes to a second extraction stage where it meets solvent containing extracted fractions from the third extraction stage in which the extraction temperature is lower than that employed in the second stage. Further separation of raffinate and extract is obtained in the second extraction stage and there is removed therefrom a second raffinate and a second extract. The extract from the second extraction stage is cooled in the same manner as the extract obtained from the first stage to obtain separation of an extract phase and a raffinate phase. As has been explained above, the extract phase obtained at this point of the process constitutes the extracting medium employed in the first extraction stage. The raffinate phase, herein, passes to the third extraction stage where it is treated in the same manner as described above, with a solvent recovered from a fourth stage operating at a lower temperature or in many cases three stages of extraction may be sufficient in which case the extraction in the third stage can be made with pure solvent. Thus we are able to obtain the maximum degree of separation of the paraffinic and non-paraffinic fractions and to conserve the quantity of solvent necessary to separate these fractions by our process.

40 It is a further object of our invention to separate the paraffinic fractions from the non-paraffinic fractions contained in hydrocarbon oils by extracting said oil in a plurality of stages with a solvent at successively lower temperatures in each stage.

45 It is a further object of our invention to countercurrently extract a hydrocarbon mixture with a solvent into a plurality of fractions in which the oil in each successive stage is extracted at a different temperature than the extraction in the previous stage and to separate from each successive stage a raffinate fraction.

50 A further object of our invention is to countercurrently extract a hydrocarbon oil mixture in successive stages with a solvent, separate a raffinate and fractions dissolved in said solvent in each successive stage, cool the solvent and dissolved fractions and separate a fraction therefrom, pass the fraction separated from the cooled solvent to a later extraction stage for extraction with solvent and pass the solvent containing the remaining dissolved fractions to an earlier extraction stage to be employed therein as solvent.

55 The accompanying figure is a schematic arrangement of one form of apparatus which we may employ to carry out our process. Referring more particularly to the figure, oil from a source, not shown, and which may previously have been treated is introduced into the lower zone of column 2 through pipe 1 along with an extracting medium introduced into the upper zone of the column through pipe 3. Owing to the difference in specific gravity of the extracting medium and oil these two liquids tend to separate. The extracting medium passes downward through the

5 extracting column and during its passage dissolves certain of the non-paraffinic fractions from the ascending column of oil. The oil from which the non-paraffinic fractions have been removed leaves the column through pipe 4 as a first raffinate.

10 The temperature of the extraction in column 2 may be relatively high and in some cases we find it desirable to maintain this temperature a few degrees below the temperature of complete miscibility of the solvent and the oil. In some cases this temperature will be 10 degrees below the point of complete miscibility, in others it is desirable that we drop the temperature 40° below this point.

15 The extracting medium and dissolved fractions are withdrawn from column 2 through line 5, valve 6 and line 7 to pump 8 which forces it through line 9 to cooler 10 where the temperature of the solution is lowered sufficiently to obtain a material separation of the oil dissolved in the extracting medium. The cooled mass in cooler 10 passes through line 11 to separator 12 where the solvent containing dissolved impurities settles out and is removed through line 13, valve 14 and line 15 to cooler 16 where it is cooled sufficiently to cause further separation of the dissolved fractions. This mass then passes to separator 17 where the solvent containing the remainder of the dissolved impurities settles out 30 and is removed through line 18, valve 19 and line 20 to storage not shown. The insoluble oil in separator 12 rises to the top and passes to the lower zone of extracting column 25 along with the insoluble oil from separator 17 which may be 35 withdrawn through line 21, pump 22 and line 23 to extracting column 25. Extracting medium enters the upper zone of column 25 through line 26 at approximately the same temperature as the oil entering the lower zone of column 25.

40 As the extracting medium moves downward through the ascending column of oil it dissolves a portion of the non-paraffinic oil present. The insoluble oil is removed from column 25 through line 27 as a second raffinate. The solution of solvent and dissolved fractions in column 25 is removed through line 28, valve 29 and line 30 to pump 31 which forces it through line 32 to cooler 33 where the temperature of the solution is lowered sufficiently to obtain a separation of the dissolved oil fractions from the solution of solvent and oil. The cooled mass then passes by means of line 35 to separator 36 where the solvent and remaining dissolved fractions settle out and are removed through line 39, valve 40 and line 41 to pump 42 which forces it through line 43 into heater 44 where it is heated to approximately the same temperature as the oil entering column 2 through pipe 1. From heater 44 this heated solvent which contains some dissolved non-paraffinic fractions passes by means of line 3 to the extracting column 2 as previously described. Due to its higher temperature and because it has been partially separated from its dissolved impurities in separator 36 its solvent power for the non-paraffinic fractions has been increased.

55 The insoluble oil in separator 36 rises to the top of the separator and passes by means of line 37 to the lower zone of column 38. Pure solvent 70 is introduced into the upper zone of column 38 through line 46 from a source not shown and at a temperature substantially the same as that of the cooled oil entering column 38 through line 37. The pure solvent passes downward through line 75

the ascending column of oil in column 38 and dissolves a portion of the impurities present in the oil. The ascending column of oil from which the impurities have been removed passes from extraction column 38 through line 45 as a third raffinate to storage not shown.

The solvent solution of extract in column 38 is removed through line 47, valve 48 and line 49 to pump 50 which forces it through line 51 to cooler 52 where the temperature of the solution is lowered sufficiently to separate a portion of the dissolved fractions. The mass then passes through line 53 to separator 54 where the insoluble oil fractions rise to the top of the column 15 and are removed as a fourth raffinate through line 55 to a source not shown.

The solvent and dissolved fractions in separator 54 settle out and are removed through line 56, valve 57 and line 58 to pump 59 which forces it through line 60 to heater 61 where its temperature is raised to a point substantially the same as that of the oil entering column 25 through line 24. From heater 61 the solvent containing some non-paraffinic fractions passes 25 by means of line 26 to the upper zone of column 25.

If desired the solvent and dissolved impurities being removed from column 38 through line 47 may be divided and a portion passed through 30 valve 62, line 63 to pump 64 which forces it through line 65 into line 60 where it meets the stream of partially purified extract coming from separator 54 through line 56, valve 57, line 58 and pump 59 and hence through the process as 35 previously described. Or if desired, valve 49 may be closed and the solvent and extract coming through line 47 may be wholly passed through valve 62 and line 63 to pump 64 which forces it through line 65 and line 60 to heater 61 from 40 which it passes by means of line 26 to extraction column 25.

As solvents one may employ B B' dichlorethyl ether, aniline, furfural, nitrobenzene, sulphur dioxide, selenium oxychloride or mixtures of these 45 solvents.

As a specific example of the method of carrying out our process with a hydrocarbon mixture consisting of paraffinic and non-paraffinic fractions and with a solvent such as B B' dichlorethyl ether, the oil to be treated at a temperature of about 110° F. enters the lower zone of extracting column 2 through line 1. Here it is countercurrently extracted with B B' dichlorethyl ether containing dissolved non-paraffinic fractions introduced into the upper zone of column 2 through line 3 at a temperature of about 110° F.

The extracted fractions and solvent are removed from column 2 to cooler 10 where the temperature is then lowered to approximately 80° F. 60 The cooled mass then passes to separator 12 where the cooled solvent and dissolved fractions settle out and pass to cooler 16 where the temperature is lowered to approximately 40° F. where a further separation of dissolved fractions takes place. The mass in cooler 16 then passes to separator 17 where the solvent and dissolved fractions settle out and are removed through line 18, valve 19 and line 20 to a still not shown, where the extract is separated from the solvent.

The insoluble fractions from the top of separators 12 and 17 enter column 25 through line 24 where they are countercurrently extracted with B B' dichlorethyl ether containing dissolved non-paraffinic fractions introduced into extraction column 25 through line 26 at a temperature 70

of approximately 80° F. The insoluble oil rises in column 25 and is removed as a second raffinate through line 27 to storage not shown.

The B B' dichlorethyl ether containing the dissolved fractions is removed from column 25 to cooler 33 where it is cooled to approximately 40° F. and then sent to separator 36. Here the B B' dichlorethyl ether containing some dissolved fractions is removed through line 39, valve 40, line 41, pump 42 and line 43 to heater 44 where 10 its temperature is raised to approximately 110° F. From heater 44 this material passes by means of line 3 to column 2.

The undissolved oil fractions in separator 36 rise and pass to the lower zone of column 38 by 15 means of line 37. Pure B B' dichlorethyl ether is introduced into the upper zone of column 38 by means of line 46 and at a temperature of approximately 40° F. The solvent being heavier than the oil settles and as it passes downward 20 dissolves non-paraffinic oil fractions from the ascending column of oil. The purified oil is removed from column 38 through line 45 as a third raffinate and sent to storage not shown.

The solvent and dissolved fractions in column 38 are then removed through line 47, valve 48, line 49, pump 50 and line 51 to cooler 52 where the temperature of the mass is lowered to 0° F. The cooled mass then passes to separator 54 where the insoluble oil rises and is removed 30 through line 55 as a fourth raffinate to storage not shown. The solution of B B' dichlorethyl ether and dissolved fractions in separator 54 is removed to heater 61 where its temperature is raised to approximately 80° F. after which it is 35 introduced into the upper zone of extraction column 25. If desired a portion of the B B' dichlor- 40 ethyl ether and dissolved fractions may be bypassed from line 47 through valve 62, line 63, pump 64, line 65 and line 60 to heater 61 and in some cases it may be desirable to close valve 48 and pass all of the solvent and extract from column 38 directly to heater 61 in which case raffinate number four is not produced.

While we have described a method of operation 45 in which the extraction in each successive stage is carried out at a decreasing temperature it is to be understood that we may employ the same temperature in each successive stage and in some cases it may be found desirable to employ increasing temperatures in each successive stage.

Where the same or increasing temperatures are employed in each successive stage it is necessary to interpose heaters in lines 1, 24, 37 and 46.

By the use of the heaters interposed in lines 1, 24, 37 and 46 and the heaters 61 and 44 it is possible to adjust the temperatures of the solvent and oil passing to columns 2, 25 and 38 to substantially the same temperatures or if desired to successively increasing temperatures. Where the same temperature in each successive stage of extraction is desired the oil passing from the heaters in lines 1, 24 and 37 and the solvent passing from the heater in line 46 and heaters 61 and 44 are at substantially the same temperature. Where an increasing temperature in successive stages is desired the temperature of the oil and solvent passing from the heaters in lines 37 and 46 to column 38 is higher than the temperature 70 of the oil and solvent passing from heater 61 and the heater in line 24 to column 25. Likewise the temperature of the oil and solvent passing to column 25 from heater 61 and the heater in line 24 is higher than the oil and solvent passing 75

to column 2 through the heater 44 and the heater in line 1.

In case cooler 52 and separator 54 are not in operation by reason of valve 48 being closed and valve 62 being open and it is desired to operate each stage at the same temperature then heater 61 functions merely as a flow line for the solvent and dissolved fractions passing from column 38 to column 25 and in case the temperature in column 25 is lower than the temperature in column 38 then heater 61 functions as a cooler for the solvent and dissolved fractions passing from the bottom of column 38 via line 47, valve 62, line 65, line 66 and line 26 to column 25.

15 The foregoing example is merely illustrative of one method of carrying out our process and is not to be construed as limiting the invention which we claim.

We claim:

20 1. A process for the production of lubricating oil from a hydrocarbon oil mixture which comprises extracting said mixture with a solvent, separating a raffinate and an extract dissolved in said solvent, cooling said solution of extract dissolved in said solvent to separate a paraffinic fraction from said solvent solution of extract, removing said paraffinic fraction from the remaining solvent solution of extract, continuously passing said cooled paraffinic fraction to a later extraction stage and extracting said fraction passed to said later extraction stage into a second raffinate and extract with a solvent.

25 2. A process for the production of lubricating oil from a hydrocarbon oil mixture which comprises extracting said mixture with a solvent into a raffinate and an extract dissolved in said solvent, separating the raffinate from the extract dissolved in said solvent, cooling said extract dissolved in said solvent to separate an insoluble fraction from the solvent and remaining dissolved fractions, removing said insoluble fraction from the solvent and remaining dissolved fractions, subsequently passing said fraction separated from said cooled extract to a later extraction stage and extracting said fraction passed to said later stage with a solvent into a plurality of fractions and passing said solvent and remaining dissolved fractions to an earlier extraction stage and extracting said oil passing to said earlier extraction stage into a plurality of fractions with said solvent containing the remaining dissolved fractions.

30 3. A process for the production of lubricating oil from a hydrocarbon oil mixture which comprises separating a raffinate and B B' dichlorethyl ether containing dissolved fractions in an earlier extraction stage, cooling said B B' dichlorethyl ether and dissolved fractions to separate an insoluble fraction therefrom, removing said insoluble fraction from said B B' dichlorethyl ether and remaining dissolved fractions, subsequently passing said insoluble fraction to a later extraction stage and extracting said insoluble fraction passing to said later extraction stage with B B' dichlorethyl ether.

35 4. A process for the production of lubricating oil from a hydrocarbon oil mixture which comprises separating a raffinate and solvent containing dissolved fractions in an intermediate extraction stage, cooling said solvent containing dissolved fractions to separate an insoluble fraction from the solvent and remaining dissolved fractions, removing said insoluble fraction from the solvent and remaining dissolved fractions, subsequently passing said insoluble fraction to a later

extraction stage and extracting said fraction passed to said later extraction stage into a plurality of fractions with a solvent and passing said solvent containing the remaining dissolved fractions to an earlier extraction stage and extracting oil passing to said earlier extraction stage into a plurality of fractions with said solvent containing the remaining dissolved fractions.

5. A process for the production of lubricating oil from a hydrocarbon oil mixture which comprises separating a raffinate and B B' dichlorethyl ether containing dissolved fractions from an intermediate extraction stage, cooling said B B' dichlorethyl ether and dissolved fractions to separate an insoluble fraction from the B B' dichlorethyl ether and remaining dissolved fractions, removing said insoluble fraction from the B B' dichlorethyl ether and remaining dissolved fractions, subsequently passing said insoluble fraction to a later extraction stage and extracting said insoluble fraction passed to said later extraction stage with B B' dichlorethyl ether, passing said B B' dichlorethyl ether containing the remaining dissolved fractions to an earlier extraction stage and extracting oil passing to said earlier extraction stage with said B B' dichlorethyl ether containing the remaining dissolved fractions.

6. A process according to claim 1 wherein the temperature of said last mentioned extraction of said paraffinic fraction recovered from the extract phase is lower than the temperature prevailing in said first mentioned extraction.

7. A process for separating a hydrocarbon mixture into a plurality of fractions which comprises commingling said oil with a selective solvent to separate a raffinate insoluble in said solvent from extract phase comprising said solvent and oil soluble therein, removing said raffinate from said extract phase, cooling said extract phase to separate an insoluble fraction from the solvent and oil fractions remaining dissolved therein, removing said insoluble fraction from said solvent and oil fractions remaining dissolved therein, cooling said last mentioned solvent and oil fractions remaining dissolved therein to separate a further insoluble fraction and continuously extracting said last mentioned insoluble fraction with a selective solvent.

8. A process for separating a hydrocarbon mixture into a plurality of fractions which comprises commingling said oil with a selective solvent to separate a raffinate insoluble in said solvent from extract phase comprising said solvent and oil soluble therein, removing said raffinate from said extract phase, cooling said extract phase to separate an insoluble fraction from the solvent and oil fractions remaining dissolved therein, removing said insoluble fraction from said solvent and oil fractions remaining dissolved therein, cooling said last mentioned solvent and oil fractions remaining dissolved therein to separate a further insoluble fraction, commingling the insoluble fractions obtained by both said cooling steps and extracting said mixture with a selective solvent.

9. A process for the separation of paraffinic from the non-paraffinic fractions of a hydrocarbon oil mixture which comprises extracting said oil with a solvent into a raffinate and fractions dissolved in said solvent, separating said solvent containing dissolved fractions from said raffinate, subsequently cooling said solvent containing dissolved fractions to separate an insoluble fraction from the solvent and remaining dissolved fractions, removing said solvent and remaining dis-

solved fractions from said insoluble fraction, thereafter passing said solvent and remaining dissolved fractions to an earlier extraction stage and extracting oil entering said earlier extraction stage into a plurality of fractions with said solvent and remaining dissolved fractions.

10. A process for the separation of paraffinic from the non-paraffinic fractions of a hydrocarbon oil mixture which comprises withdrawing solvent containing dissolved fractions from a later extraction stage, cooling said solvent containing dissolved fractions to separate an insoluble fraction therefrom, separating said solvent and remaining dissolved fractions from said insoluble fraction, subsequently passing said solvent containing remaining dissolved fractions to an earlier extraction stage and extracting oil passing to said earlier extraction stage into a plurality of fractions with said solvent containing remaining dissolved fractions.

11. A process for the production of lubricating oil from a hydrocarbon oil fraction which comprises extracting said mixture with a solvent, separating a raffinate and an extract dissolved in said solvent, cooling said solution of extract and solvent to separate a paraffinic fraction from said

cooled solution of extract, removing said insoluble paraffinic fraction from the remaining cooled solution of extract, subsequently passing said cooled solution of extract through a heater to raise the temperature of said solution and passing said heated solution of solvent and extract to an earlier extraction stage to be employed therein as the extracting medium.

12. A process for the separation of paraffinic and non-paraffinic fractions from an oil containing the same which comprises commingling said oil in an extraction stage with a selective solvent, forming a raffinate phase comprising relatively paraffinic oil fractions and an extract phase comprising selective solvent and relatively non-paraffinic fractions, separating said phases, removing a paraffinic oil fraction from the extract phase, returning the selective solvent containing the remaining dissolved fractions to an earlier extraction stage, and extracting oil passing to said earlier extraction stage with the selective solvent containing the remaining dissolved fractions.

DAVID R. MERRILL. 25  
PHILIP SUBKOW.